

United States Patent [19]  
Ricks

[11] B 3,915,667  
[45] Oct. 28, 1975

[54] ABRASION RESISTANT COATING FOR  
ALUMINUM BASE ALLOY AND METHOD

[75] Inventor: **Herbert E. Ricks**, Pittsburgh, Pa.

[73] Assignee: **Westinghouse Electric Corporation**,  
Pittsburgh, Pa.

[22] Filed: Sept. 20, 1973

[21] Appl. No.: 399,766

[44] Published under the Trial Voluntary Protest  
Program on January 28, 1975 as document no.  
B 399,766.

[52] U.S. Cl. .... 29/197; 117/71 M; 204/33

[51] Int. Cl.<sup>2</sup> .... C23B 5/00; C23B 5/22

[58] Field of Search .... 117/71 M; 204/33, 40, 38 B;  
29/197

[56] References Cited

UNITED STATES PATENTS

2,624,684 1/1953 Heiman..... 204/38 A X

|           |         |                                 |
|-----------|---------|---------------------------------|
| 2,654,701 | 10/1953 | Calderon et al. .... 204/38 A X |
| 2,995,814 | 8/1961  | Chamness ..... 204/33 X         |
| 3,108,006 | 10/1963 | Kenedi et al. .... 204/33 X     |
| 3,455,014 | 7/1969  | Beyer ..... 204/40 X            |

Primary Examiner—L. Dewayne Rutledge

Assistant Examiner—Arthur J. Steiner

Attorney, Agent, or Firm—L. P. Johns

[57]

ABSTRACT

The method for applying an abrasion resistant coating on the surface of an aluminum or aluminum alloy conductor. After cleaning the conductor surface to remove dirt, grease, and oxides and to make the surface uniformly active, a plurality of coatings of metals are applied including an inner coating of tin or zinc, intermediate coatings of bronze or copper, and nickel, and an outer coating of tin or silver.

3 Claims, No Drawings

## ABRASION RESISTANT COATING FOR ALUMINUM BASE ALLOY AND METHOD

### CROSS REFERENCE TO RELATED APPLICATION

This application is related to the invention disclosed in the application of Julius Toth and Edward M. Walker, Ser. No. 364,173, filed May 25, 1973.

### BACKGROUND OF THE INVENTION

#### 1. Field of the Invention

This invention relates to an abrasion resistant coating for an aluminum and aluminum alloy conductor and to a method for applying the coating.

#### 2. Description of the Prior Art

Since 1945, the substitution of aluminum for copper as electrical conductor material has continually increased until at the present time over 50% of the conductors are made of aluminum. This trend is due to the almost unlimited availability of aluminum and its much lower cost compared to copper. The substitution of aluminum for copper in bus bars, however, can result in a cost saving only if a low cost process for plating the contact joints is available. The ever present high-resistivity oxide coating on the aluminum must be replaced with a high conductivity coating such as silver plate if the aluminum conductors are to be treated like copper conductors with respect to bolting and unbolting during assembly. However, for stab type contacts to bus bars in bus duct and load center apparatus, it is necessary to have the aluminum coated with a good wear resistant coating such as copper or nickel plus a coating such as silver, tin, or cadmium for lubrication and low contact resistance.

The application of protective coatings for various purposes on the surface of members composed of aluminum and aluminum alloys is well-known in the art such as disclosed in U.S. Pat. Nos. 2,377,606; 2,947,639; and 3,274,021. Generally, those patents disclosed a method for providing a tightly adherent tin coating on an aluminum surface.

Where specific environmental problems are incurred, additional protection is necessary. In the past a coating consisting of layers of zinc, copper, and silver plating on aluminum bus bars has left much to be desired for environmental protection; improved corrosion resistance in specialized areas has been indicated.

Associated with the foregoing has been a problem of fretting due to either mechanical wear or corrosion. In one form fretting is wear resulting from oscillating or vibratory motion of a limited amplitude. Another form of fretting results from actual wear, frictional changes, variations in electrical resistances, electrical noise, and fatigue failure. Aluminum is particularly susceptible to fretting corrosion which is the formation of hard abrasive oxides ( $Al_2O_3$ ) as debris and by an excessive rate of oxygen absorption. As a result, there has been a problem of providing aluminum members, such as bus bars or conductors, with a protective coating of a suitable type of which abrasion and corrosion are avoided.

### SUMMARY OF THE INVENTION

Generally, it has been found in accordance with this invention that the foregoing problems may be overcome by providing an aluminum conductor or bus bar with a multiple layered coating of various metals applied in a given sequence, which sequence consists es-

sentially of an inner layer of tin or zinc, intermediate layers of bronze or copper, and nickel, and an outer layer of either tin or silver. Where the conductor or bus bar is subject to vibrations, an outer coating of silver instead of tin is preferred.

The invention also comprises a method for applying the several layers in the indicated sequence.

### DESCRIPTION OF THE PREFERRED EMBODIMENT

10

According to the present invention in practice the new method is carried out in the following sequential manner:

1. Preliminarily cleaning the surface of an aluminum member to be coated with a caustic solution to remove oxides, dirt, grease, and the like;
2. Rinsing the surface in water;
3. Cleaning the surface with an acid;
4. Rinsing the member in water;
- 20 5. Applying an inner coating of tin or zinc to the surface;
6. Applying a copper-base alloy to the tin coating or copper strike on the zinc coating;
7. Rinsing the member in water;
8. Applying a coating of nickel on the copper-base alloy or copper coating;
9. Rinsing the member in water;
10. Applying an outer coating of tin or silver on the coating of nickel, and

30

11. Rinsing the member in water and air drying

The method is applicable to pure aluminum and a wide range of aluminum alloys such as aluminum alloy numbers 6061, 6101, 2024, 5052, 7075, 356, 360, and 380.

- 35 12. The first step comprises cleaning the surface with a caustic solution to remove oxides, dirt and the like, and removes about  $\frac{1}{2}$  to 1 mil of aluminum surface. The preferred solution for this purpose is about 8 to 10 ounces of sodium hydroxide per gallon of water at 180°F which is applied to the aluminum surface for a time of from about  $\frac{1}{4}$  to 1 minute. Other alkali metal hydroxides such as potassium hydroxide may be used. A chelating agent is preferably added to the solution to slow down the action. A common chelating agent is ethylenediaminetetraacetic acid (EDTA). The advantage of the chelating agent is to maintain the material removed from the aluminum surface in solution.

- 40 13. The second step is a water rinse to remove all traces of the caustic solution of the first step because the third step involves an acid solution. After the member is cleaned with a caustic solution, a thick viscous coating or smut of sodium zincate ( $Na_2ZnO_2$ ) adheres to the member. This coating is removed better by a double rinse in water.

- 45 14. The third step is a surface cleaning or desmutting operation with an acid solution such as a 1:1 mixture of nitric acid (67%) in water for the purpose of deoxidizing and removing impurities in aluminum such as iron and manganese. Although it is not necessary, about 1 to 5% hydrofluoric acid is preferably added to make the aluminum surface more uniformly active and to prevent blistering of some subsequently deposited metal, such as tin. The blistering often occurs due to poor metal preparation.

- 50 15. The fourth step is another rinse in water to remove all traces of acid of the previous rinse, because the next step involves an alkaline bath.

The fifth step has the dual purpose of activating the aluminum surface and depositing a thin layer of tin or zinc. In this step, where the thin layer is tin, the aluminum member is immersed in aqueous solution, the primary constituent of which is at least one tin-containing compound selected from the group consisting of a stannate of an alkali metal, such as sodium stannate and potassium stannate, together with a chelating agent such as EDTA. The composition of the solution is shown in Table I as follows:

Table I

| Activating & Immersion Tin Plating Bath                                                                                                        |                                                       |                   |
|------------------------------------------------------------------------------------------------------------------------------------------------|-------------------------------------------------------|-------------------|
| Constituent                                                                                                                                    | (Ounces per gallon of water)<br>Preferred Composition | Range Composition |
| Na <sub>2</sub> SnO <sub>3</sub> ·H <sub>2</sub> O<br>and/or<br>K <sub>2</sub> SnO <sub>3</sub> ·H <sub>2</sub> O<br>Chelating Agent<br>(EDTA) | 11<br>6                                               | 8-14<br>1-10      |

The constituents, sodium stannate and potassium stannate, may be used either alone or mixed to make up the required composition. Sodium stannate and potassium stannate used here and in subsequent steps may be used either in the anhydrous or the trihydrate form; it being immaterial, because the operating conditions required the solution to be maintained at an elevated temperature of from 75° to 85°F with a preferred temperature of 80°F. The immersion time may range from 15 to 45 seconds with a preferred time of 30 seconds. A partial or wholly substitute chelating agent is preferably used for stabilizing the time to prevent it from settling to the bottom of the container. It is a mixture of zinc acetate, Zn (C<sub>2</sub>H<sub>3</sub>O<sub>2</sub>)<sub>2</sub>, in an amount of about 2 ounces per gallon of water and m-cresolsulfonic acid in the amount of about 4 ounces per gallon of water. Thus, by step 5 the surface of the aluminum member is completely activated and the protective layer of tin is deposited. The weight of tin deposited varies from about 0.1 to 0.3 mg/in<sup>2</sup>.

On the other hand in step 5 where the thin layer is zinc instead of tin, the aluminum member is immersed in an aqueous solution having at least one zinc-containing compound, such as zinc oxide and sodium hydroxide. The immersion time may range from 15 to 45 seconds with a preferred time of about 30 seconds at a temperature of from 75° to 85°F with a preferred temperature of 80°F. The composition of the zinc solution is shown in Table II as follows:

Table II

| Activating & Zinc Plating Bath |                                                       |                   |
|--------------------------------|-------------------------------------------------------|-------------------|
| Composition                    | (Ounces per gallon of water)<br>Preferred Composition | Range Composition |
| NaOH                           | 60                                                    | 50-70             |
| ZnO                            | 13                                                    | 11-14             |
| Chelating Agent                | 6                                                     | 1-10              |

The chelating agent is preferably used as a stabilizer of the solution.

The sixth step is the application of a coating of copper or a copper-base alloy. Where in step 5 tin is applied, a coating of a copper-base alloy such as a bronze

strike is applied on the tin in step 6. However, where zinc is applied in Step 5, a copper strike is applied in step 6. Where tin is applied, a rinse between steps 5 and 6 is unnecessary because the solutions of both steps are alkaline. But where zinc is applied, a rinse is preferred before the application of copper. The sixth step is accomplished by immersing the aluminum member into an electrolyte consisting essentially of a stannate of an alkali metal such as sodium stannate and copper cyanide. A partial or complete substitute for sodium stannate may be potassium stannate. The constituents and the amounts used for the bronze strike are shown in Table III as follows:

Table III

| Bronze Strike                                                                 |                                                       |                   |
|-------------------------------------------------------------------------------|-------------------------------------------------------|-------------------|
| Constituent                                                                   | (Ounces per gallon of water)<br>Preferred Composition | Range Composition |
| Na <sub>2</sub> SnO <sub>3</sub><br>and/or<br>K <sub>2</sub> SnO <sub>3</sub> | 7-11                                                  |                   |
| CuCN                                                                          | 5                                                     | 4.5-5.5           |
| KCN (Free)                                                                    | 4                                                     | 3-5               |
| KOH (Free)                                                                    | 9                                                     | 7-11              |
|                                                                               | 1.5                                                   | 1-1.75            |

The electrolyte solution consisting of the constituents listed in Table III includes potassium cyanide (KCN) and potassium hydroxide (KOH) which increase the conductivity and efficiency of the electrolyte and improve the erosion of the copper and tin anodes, thereby reducing the current loss and maintaining the desired electrolyte temperature. In addition, by improving anode corrosion, the amount of makeup of the constituents sodium stannate and potassium stannate as well as copper cyanide is reduced.

The operating conditions of the bronze strike step are shown in Table IV, as follows:

Table IV

| Operating Conditions       |            |               |
|----------------------------|------------|---------------|
| Condition                  | Preferred  | Range         |
| Time                       | 30 seconds | 15-45 seconds |
| Temperature                | 140°F      | 135-145°F     |
| Cathode Current<br>density | 30 ASF     | 20-30 ASF     |
| Anode Current<br>density   | 15 ASF     | 10-20 ASF     |
| pH                         | 11.75      | 11.5-12.5     |
| Anodes                     | copper     |               |

The thickness of the bronze coating may vary from about 0.00001 to 0.00003 inch.

Where the sixth step is an application of a coating of copper instead of bronze, the constituents and other parameters of the copper solution are listed in Table V as follows:

Table V

| Copper Strike Conditions |                          |                      |
|--------------------------|--------------------------|----------------------|
| Constituent              | Preferred<br>Composition | Range<br>Composition |
| CuCN                     | 5.6 oz/gal               | 4-6 oz/gal           |
| NaCN                     | 6.4 oz/gal               | 5-7 oz/gal           |
| Rochelle Salt            | 8 oz/gal                 | 6-10 oz/gal          |
| Temperature              | 120-130°F                | 115-135°F            |

Table V-Continued

| Copper Strike Conditions |                       |                   |
|--------------------------|-----------------------|-------------------|
| Constituent              | Preferred Composition | Range Composition |
| Current Density          | 25 ASF                | 20-30 ASF         |
| pH                       | 10                    | 9.8-10.7          |
| Anodes                   | Copper                |                   |

If the temperature is too high (above 135°F), the zinc layer is dissolved off. If the pH is too high—above 10.5, the zinc layer is dissolved by the alkali.

The seventh step is a water rinse for the purpose of removing the bronze or copper strike solutions and for preventing contamination of the nickel plate solution which is the eighth step.

The eighth step is the application of a relatively thick layer of nickel on the bronze or copper strike. The aluminum member is immersed in electrolyte having the constituents listed in Table VI as follows:

Table VI

| Nickel Plate       |                                           |           |
|--------------------|-------------------------------------------|-----------|
| Constituent        | (Ounces per gallon of water)<br>Preferred | Range     |
| Nickel Sulfamate   | 50-60                                     | 20-70     |
| Boric Acid         | 4-4.5                                     | 3.5-5     |
| Anti-Pitting Agent | 0.06                                      | 0.05-0.07 |

The thickness of the resulting nickel plate ranges from about 0.0001 to 0.0005 inch, the preferred thickness being 0.0002 inch. The operating conditions for the electrolyte bath are listed in Table VII as follows:

Table VII

| Operating Conditions |           |         |
|----------------------|-----------|---------|
|                      | Preferred | Range   |
| pH                   | 5-5.5     | 3-5.5   |
| Temperature °F       | 120       | 110-130 |
| Current              | 30 ASF    | 30-40   |

Although nickel plated from the nickel sulfamate is disclosed, nickel may be plated from other solutions such as:

| Watts Type Bath         |                |  |
|-------------------------|----------------|--|
| High-pH                 |                |  |
| Nickel sulfate          | 32 oz/gal      |  |
| Nickel chloride         | 6 oz/gal       |  |
| Boric acid              | 4 oz/gal       |  |
| pH                      | 4.5-6.0        |  |
| Temperature             | 115-160°F      |  |
| Current density         | 20-100 ASF     |  |
| Hard Nickel Bath        |                |  |
| Nickel sulfate          | 24 oz/gal      |  |
| Ammonium chloride       | 3.3 oz/gal     |  |
| Boric acid              | 4.0 oz/gal     |  |
| pH                      | 5.6-5.9        |  |
| Temperature             | 110-140°F      |  |
| Current density         | 25-50 ASF      |  |
| Sulfamate Chloride Bath |                |  |
| Nickel sulfamate        | 80 oz/gal      |  |
| Nickel Chloride         | 0.6-0.7 oz/gal |  |
| Boric acid              | 5.3 oz/gal     |  |
| pH                      | 4.5            |  |
| Temperature             | 140-160°F      |  |

-Continued

| Watts Type Bath |                                 |                   |
|-----------------|---------------------------------|-------------------|
| High-pH         |                                 |                   |
| 5               | Current density                 | All-Chloride Bath |
|                 | Nickel Chloride                 | 40 oz/gal         |
|                 | Boric acid                      | 4 oz/gal          |
|                 | pH                              | 4.5               |
|                 | Temperature                     | 130-160°F         |
|                 | Current density                 | 25-100 ASF        |
| 10              | Fluoborate Bath                 |                   |
|                 | Nickel fluoborate               | 40 oz/gal         |
|                 | Boric acid                      | 4 oz/gal          |
|                 | pH                              | 4.5               |
|                 | Temperature                     | 100-170°F         |
|                 | Current density                 | 25-100 ASF        |
|                 | The ninth step is a water rinse |                   |

The tenth step is the application of tin or silver as preferred. A rinse in two baths of cold water is required before plating of tin or silver.

Where the choice is tin, the copper plated aluminum member is immersed into the plating solution having the formula and operating conditions set forth in Tables VIII and IX as follows:

Table VIII

| Tin Plate            |                                                       |                   |
|----------------------|-------------------------------------------------------|-------------------|
| Constituent          | (Ounces per gallon of water)<br>Preferred Composition | Range Composition |
| KOH                  | 2                                                     | 1-4               |
| $K_2SnO_3$ and/or    |                                                       |                   |
| $Na_2SnO_3$          | 28                                                    | 26-28             |
| Tin metal equivalent | 10.6                                                  | 10-11             |

Table IX

| Operating Conditions                                                                  |                     |           |
|---------------------------------------------------------------------------------------|---------------------|-----------|
|                                                                                       | Range               | Preferred |
| Temperature °F                                                                        | 130-180             | 140°F     |
| Voltage                                                                               | 3-6                 |           |
| Current density                                                                       | 30-160 ASF          | 75        |
| Anode to Cathode ratio                                                                | Never more than 1:2 |           |
| Time to deposit .0001 to .0006 in. of plating at recommended current density, minutes | 2-4                 | 2         |

The thickness of the outer tin plate or coating may range from 0.0001 to 0.0006 inch, the preferred thickness being 0.0005 inch.

Where the outer plating or coating is silver instead of tin, the copper-plated aluminum member is placed in the silver plating electrolyte having a formula and control conditions as set forth in Tables X and XI as follows:

Table X

| Silver Plate |                                           |         |
|--------------|-------------------------------------------|---------|
| Constituent  | (Ounces per gallon of water)<br>Preferred | Range   |
| $AgCN$       | 0.7                                       | 0.5-0.8 |
| $Na_2CN$     | 9                                         | 8-10    |

Table XI

| Operating Conditions |            |           |
|----------------------|------------|-----------|
|                      | Preferred  | Range     |
| pH                   | 10.9       | 10.2-11.5 |
| Time                 | 10 seconds | 5-60      |
| Temperature          | 85°F       | 70-105    |
| Current Density      | 20         | 15-25     |

A silver plating or coating thickness of from 0.00003 to 0.00005 inch is normally deposited in about 10 seconds for the indicated current density. As in the preceding deposition such as for the copper and tin, the cathode is the aluminum member held stationary in the electrolyte. The anode is composed of copper, tin, or silver depending upon the metal being deposited.

The eleventh step is the final rinse in hot water after which the member is dried in hot air.

It is noted that although the several rinse steps are preferably used to prevent early contamination of the plating solutions, the rinsing steps may be omitted for the purpose of this invention.

The resulting protective coating provided in the method set forth above provides a corrosion and abrasion resistant plating for stabs or bus ducts when bus bars are subjected to 30,000 consecutive abrasion tests, i.e. involving sliding wear.

Wearing tests on aluminum bus bars with and without nickel coating were made for composition. The results of the wear tests are shown in Table XII as follows:

Table XII

| Coating Process                                                                                       | No. of<br>Stab Insertions <sup>a</sup><br>Before Coating<br>Wore Through to<br>Bare Aluminum <sup>b</sup> |
|-------------------------------------------------------------------------------------------------------|-----------------------------------------------------------------------------------------------------------|
| 1. (Alstan 70 process): immersion<br>tin + bronze strike +0.0004 inch<br>copper + 0.00005 inch silver | 200                                                                                                       |
| 2. Same as above but with 0.0002<br>inch nickel + 0.00005 inch silver                                 | 350                                                                                                       |
| 3. Zincate process-immersion Zinc<br>+ 0.00004 inch copper + 0.0005<br>inch silver                    | 275                                                                                                       |

35

40

45

50

55

60

65

4. Same as above but 0.0002 inch  
nickel + 0.00005 inch silver

400

<sup>a</sup> 135 ampere stab contacts plated with 0.00005 inch silver

<sup>b</sup> A 5% solution of caustic soda was used to determine the presence of bare aluminum. Vigorous gassing occurred when this solution was applied to the worn through plate on bare aluminum.

The multiple layered coating of this invention satisfies the foregoing problem of fretting with attendant problems. The bronze or copper plating provides a suitable substrate for the nickel strike. The nickel plating has a tri-fold advantage including the establishment of a base for the silver or tin which is subsequently applied, corrosion prevention, and providing a harder base for sliding friction on the stab surface as indicated in Table XII. Silver serves as a lubricant and resists fretting better than tin and does it with a thinner coating.

What is claimed is:

1. A composite article comprising an aluminum alloy member having an abrasion resistant coating on the surface thereof, said coating consisting essentially of an inner layer of a metal selected from the group consisting of tin and zinc, a first intermediate layer of a metal selected from a group consisting of copper and bronze, a second intermediate layer of nickel, and an outer layer of a metal selected from a group consisting of tin and silver.

2. The layer of claim 1 in which the inner coating is tin, the intermediate layer is bronze and the outer layer is tin.

3. The layer of claim 1 in which the inner layer is zinc, the intermediate layer is copper and the outer coating is silver.

\* \* \* \* \*